

# United States Patent Office.

LORENZO SIBERT, OF MOUNT SOLON, VIRGINIA.

*Letters Patent No. 79,152, dated June 23, 1868.*

## IMPROVEMENT IN THE MANUFACTURE OF IRON AND STEEL.

The Schedule referred to in these Letters Patent and making part of the same.

TO ALL WHOM IT MAY CONCERN:

Be it known that I, LORENZO SIBERT, of Mount Solon, in the county of Augusta, and State of Virginia, have invented a new and useful Improvement in the Manufacture of Iron and Steel, resulting in a product which I call the "Sibert Alloy;" and I do hereby declare the following to be a full, clear, and exact description thereof, which will enable others skilled in the art to make and use the same.

My invention or discovery consists of a new and improved method of treating iron ores, in the process of reduction, in an ordinary blast-furnace, so as to produce the "Sibert alloy," and then to apply said "alloy" to the various purposes for which cast and wrought iron and steel are used in the arts, and for most of which it is well suited. My process is substantially as follows:

In a common iron-furnace, and in connection with the ordinary lime flux, I use a compound of manganese and common salt. The proportions in which these materials are used vary according to the quantity of the ores to be reduced and of the metal to be produced, and they modify to some extent the proportion of lime to be used, as the experience of the founder will readily ascertain. I have used with the best results about five hundred pounds of manganese and ten or fifteen pounds of salt for a ton of metal produced. The manganese is used in the form of black oxide or of "wad," and the salt is best applied in the form of a brine, poured over the manganese.

In connection with the use of the compound flux above described, and as a means of securing uniformity in the metal produced, I increase or diminish the blast used in the reduction of the ore without changing the binder of the furnace. The experience of the founder will enable him to regulate this use of the blast so as to secure a uniform run of metal of any grade desired.

If, by any mistake in the flux, or in the use of the blast, the metal in the hearth is found to be below the grade desired, it may be brought up to the standard by putting in at the dam more or less of the same metal prepared for the purpose, and charged with carbon in excess. When the crucible of the furnace is about two-thirds full of molten metal, I stir in, with a "quash," about one pound of Epsom salts to the ton of metal, and let it remain for about three-quarters of an hour before the metal is run out. This is used as a purifier.

The metal thus produced, if intended to be recast in a foundry, may be run from the furnace into sand. When recast, it should be again treated with the same flux and process, the quantities and proportions being varied according to the grade of the metal used, and the result desired. I have used with success in recasting about sixty pounds of manganese, five pounds of salt, and three-quarters of a pound of Epsom salts to a ton of metal. If intended to be hammered or rolled, it should be run into hot metallic moulds, and annealed by gradual cooling.

When intended for railroad-iron, the metal should be of the highest grade, and should be run at once into red-hot metallic moulds. It should be kept for eight or ten hours at an annealing-heat in the moulds, and, if desired, the face of the rail may be hardened by chilling.

Having thus described my invention, what I claim as new, and desire to secure by Letters Patent, is—

1. The use of manganese, in combination with common salt, substantially in the manner and for the purposes herein set forth.
2. I claim the use of Epsom salts in the treatment of iron in the furnace, for the purpose of purifying the iron.
3. The method of treatment herein described for reducing and purifying the ores and the metal, and for securing uniformity in the quantity of the metal produced.

LORENZO SIBERT.

Witnesses:

CHAS. A. PETTIT,  
SOLON C. KEMON.